

June 27, 1967

P. A. LAWRENCE

3,328,286

CATALYTIC REFORMING OF PETROLEUM HYDROCARBONS WITH  
PLATINUM ON A LOW BENZENE CHEMISORPTION ALUMINA

Filed July 8, 1964

4 Sheets-Sheet 1



INVENTOR,  
PAUL ANTHONY LAWRENCE

BY

MORGAN, FINNEGAN, DURHAM & PINE

ATTORNEYS

June 27, 1967

P. A. LAWRENCE

3,328,286

CATALYTIC REFORMING OF PETROLEUM HYDROCARBONS WITH  
PLATINUM ON A LOW BENZENE CHEMISORPTION ALUMINA

Filed July 8, 1964

4 Sheets-Sheet 2

FIG. 3.



INVENTOR,  
PAUL ANTHONY LAWRENCE  
BY  
MORGAN, FINNEGAN, DURHAM & PINE  
ATTORNEYS

June 27, 1967

P. A. LAWRENCE

3,328,286

CATALYTIC REFORMING OF PETROLEUM HYDROCARBONS WITH  
PLATINUM ON A LOW BENZENE CHEMISORPTION ALUMINA

Filed July 8, 1964

4 Sheets-Sheet 3

FIG. 4.



INVENTOR,  
PAUL ANTHONY LAWRENCE

BY

MORGAN, FINNEGAN, DURHAM & PINE

ATTORNEYS

June 27, 1967

P. A. LAWRENCE

3,328,286

CATALYTIC REFORMING OF PETROLEUM HYDROCARBONS WITH  
PLATINUM ON A LOW BENZENE CHEMISORPTION ALUMINA

Filed July 8, 1964

4 Sheets-Sheet 4

FIG. 5a.



FIG. 5b.



INVENTOR,  
PAUL ANTHONY LAWRENCE

BY  
MORGAN, FINNEGAN, DURHAM & PINE  
ATTORNEYS

1

3,328,286  
**CATALYTIC REFORMING OF PETROLEUM HYDROCARBONS WITH PLATINUM ON A LOW BENZENE CHEMISORPTION ALUMINA**

Paul Anthony Lawrence, Sunbury-on-Thames, Middlesex, England, assignor to The British Petroleum Company, London, England, a corporation of England

Filed July 8, 1964, Ser. No. 381,036

Claims priority, application Great Britain, Aug. 2, 1963, 30,671/63; Feb. 27, 1964, 8,185/64  
 19 Claims. (Cl. 208—65)

This invention relates to the catalytic reforming of hydrocarbons using a platinum group metal-alumina catalyst.

Catalytic reforming using a platinum-alumina catalyst is a well-established petroleum conversion process which is used to upgrade gasoline and naphtha boiling range hydrocarbons (i.e. C<sub>5</sub> to 204° C. fractions) to products of increased aromatic content. These products can be used either as high octane gasolines or as sources of aromatics.

A variety of aluminas have been proposed as supports for the platinum group metal but the predominant emphasis has been on aluminas which show appreciable catalytic activity in themselves, particularly hydrocracking activity. Hydrocracking activity is, in its turn, related to the acidity of the aluminas and consequently the normal commercial catalysts have a moderate to high acidity. The emphasis on catalysts with hydrocracking activity is believed to stem from a desire to achieve high octane numbers at moderate temperatures. An alternative approach, however, is to rate a catalyst in terms of the yield of product obtained for a given octane number. Thus, the present invention is concerned with the use of a catalyst which gives products with an improved yield-octane number relationship.

There is accordingly disclosed a process for the catalytic reforming of hydrocarbons which comprises contacting a gasoline or naphtha in the presence of hydrogen and under reforming conditions, with a catalyst of a platinum group metal on a support consisting of an alumina having a reversible benzene chemisorption, as hereinafter specified, of up to 5  $\mu$ moles/g.

The invention further consists in a process for the catalytic reforming of hydrocarbons which comprises contacting a gasoline or naphtha in the presence of hydrogen and under reforming conditions, first with a catalyst of a platinum group metal on a support consisting of an alumina having a reversible benzene chemisorption of up to 5  $\mu$ moles/g., and then with a catalyst of a platinum group metal on a support which is more acidic than the aforementioned alumina.

Preferably the reversible benzene chemisorption is at least 0.3  $\mu$ mole/g.

The reversible benzene chemisorption is a measure of acidity, low figures indicating a low acidity. The measurement of the benzene chemisorption of an alumina involves contacting the alumina with benzene vapor at a low partial pressure and a fixed temperature, and measuring the amount of vapor adsorbed and desorbed. The amount of the benzene chemisorbed may vary with the test conditions used, and in particular with the partial pressure of the benzene vapor and the temperature. It is thus necessary to standardize the conditions, and for the purpose of the present invention the partial pressure used is 0.1 mm. Hg, and the temperature 193° C.

One description of a suitable technique for measurement of benzene adsorption and an apparatus therefor is to be found in a paper by R. C. Pitkethly and A. G. Goble, entitled "The Adsorption of Benzene on Supported Platinum Catalysts," and published in "Actes du Deuxieme Congres International de Catalyse," Paris, 1960, vol. 2, at

2

page 1851. Adsorption at low partial pressures is normally attributable to chemisorption with a relatively small contribution from physical adsorption and the apparatus for measuring it has three principal sections, viz.

- 5 (a) A vapor introduction device;  
 (b) A holder for the solid to be tested;  
 (c) A vapor detector.

The vapor introduction device has a source of carrier gas, for example nitrogen or hydrogen, a container for the material to be adsorbed and a valve allowing either the gas alone or gas containing very small quantities of the material to be adsorbed to pass over the solid. The holder which contains the catalyst or catalyst support is capable of being held at a constant temperature over a wide temperature range. Gas passing over the catalyst then goes via the sampling valve to the vapor detector which may be a hydrogen flame-ionization detector. The detector system may have gas chromatographic columns if the relative rates of adsorption of different materials are to be determined or if reaction is likely under the conditions of test and the composition of the reaction product is to be determined. This is not likely to apply to the present invention.

By passing a stream of gas containing material to be adsorbed over the catalyst or catalyst base to be tested and measuring the difference between the amount of material fed to the catalyst or catalyst base and the amount passing to the detector, the amount of material adsorbed can be determined, after a small correction for dead space in the system. If the flow of material is then discontinued and gas alone is passed over the catalyst, the amount of material which can be desorbed can also be determined. The amount desorbed is known as the reversible adsorption; the difference between the amounts adsorbed and desorbed is known as the irreversible adsorption.

The carrier gas for the benzene vapor should be inert to alumina and is, preferably, nitrogen.

The aluminas to be tested are desirably given a standard pretreatment to bring them to a standard chemical and physical state and eliminate any effects which could be due, for example, to different water contents. Prolonged heating in an inert atmosphere is preferred, for example heating between 100–800° C. in dry nitrogen for 1 to 75 hours. A particularly preferred pretreatment is heating at 500° C. for 16 hours in dry nitrogen.

Preferably the test is carried out on aluminas alone. However since the catalysts also contain a platinum group metal it may be convenient or necessary, in certain circumstances, to carry out the test on aluminas which already have a platinum group metal composited therewith. If a platinum group metal is present, this will also adsorb the benzene. However this platinum group metal adsorption is irreversible, and can, therefore, be distinguished from the reversible adsorption due to the alumina.

55 Aluminas having a reversible benzene chemisorption of up to 5  $\mu$ moles/g. are hereinafter termed "low-acidity aluminas." They may suitably be prepared from the alumina hydrate known generally as pseudoboehmite. This hydrate is characterized by a poorly crystalline form showing a diffuse boehmite type X-ray diffraction pattern. On calcination under normal conditions (e.g., temperatures of 450°–650° C.) the hydrate is converted to a poorly crystalline alumina which some authorities refer to as gamma-alumina and some as eta-alumina. The second nomenclature is preferred and will be used in describing the present invention.

The aluminas used should be of high purity, having in particular an alkali metal content of less than 0.01% wt., and a preferred method of preparation is to form pseudoboehmite by hydrolyzing an aluminium alcoholate at less than 70° C. under conditions such that the normal crys-

tallization sequence amorphous→pseudoboehmite→bayerite does not proceed beyond the pseudoboehmite stage. A particularly suitable hydrolyzing medium is an aqueous solution of hydrogen peroxide. The concentration of hydrogen peroxide may conveniently be in the range 1-30% wt., increase in the concentration under otherwise similar conditions, tending to decrease the degree of crystallinity of the pseudoboehmite. The hydrolyzing temperature may be within the range 0° C. to 70° C., preferably from 0° C. to 40° C.

The aluminium alcoholate may be prepared in any convenient manner. One suitable method comprises reacting aluminium metal with an alcohol, preferably in the presence of a small quantity of mercury or of a mercury compound. A preferred alcoholate is aluminium isopropoxide.

The aluminium alcoholate may, if desired, be dissolved in a hydrocarbon solvent, which may be a pure hydrocarbon, for example an aromatic hydrocarbon, such as benzene or toluene, or a paraffinic or cycloparaffinic hydrocarbon, or the solvent may be a mixture of hydrocarbons, for example a petroleum fraction boiling in the gasoline or naphtha range (i.e., up to 204° C.). Preferably the solvent has an appreciably greater solvent power for the alcohol produced by the hydrolysis than the water used as hydrolyzing medium, thereby facilitating the recovery or re-use of the alcohol. The presence of the hydrocarbon solvent appears to facilitate the reaction between the alcoholate and water.

After the hydrolysis the hydrated alumina is separated from the other materials present. The hydrocarbon solvent, if used, will contain some of the liberated alcohol and this may be decanted. The aqueous phase may be separated by filtering and washed as necessary.

No ageing of the wet hydrated alumina is necessary. However, if it is not possible to carry out the next step of catalyst preparation immediately (i.e., if there is unavoidable ageing) this will not be deleterious, since a particular feature of the pseudoboehmite hydrogels used in the present invention is their stability.

The wet alumina hydrate may be dried at, for example 100-110° C. and calcined to alumina under normal conditions (i.e., temperatures of 250 to 650° C., preferably 250 to 550° C.).

The preferred platinum group metal is platinum and the platinum group metal may be added by known techniques at any convenient point in the alumina preparation. Preferably it is added to the wet alumina hydrate and for this purpose the alumina hydrate filter cake may be redispersed as a slurry and a platinum group metal compound added. The platinum group metal compound composited with the hydrated alumina is preferably a platinum group metal sulphide and a particularly preferred method of forming this is to add a solution of a platinum group metal compound, for example chloroplatinic acid, to the hydrogel and to precipitate platinum sulphide by the addition of hydrogen sulphide in, for example, the form of a saturated aqueous solution. The amount of platinum group metal composited with the hydrated alumina should be sufficient to give a finished catalyst containing from 0.01 to 5% wt., preferably from 0.1 to 1% wt., of platinum group metal. The platinum group metal-alumina hydrate composite may then be filtered, and dried and calcined as indicated above.

The benzene chemisorption technique used to determine the suitability of aluminas for use in the present invention is illustrated with reference to the accompanying drawings, in which:

FIGURE 1 is a diagrammatic flow sheet of an apparatus for measuring benzene chemisorption, and

FIGURE 2 is a typical record obtained with the apparatus of FIGURE 1.

In FIGURE 1, nitrogen from a source 1 is passed through a pressure regulator 2, controlled with reference to a pressure gauge 3, to impurity traps 4 and 5 containing,

respectively, manganous oxide to remove oxygen and a 4 A molecular sieve to remove water. After the traps the nitrogen line is split, one branch 6, having a valve 7 in it, passing to the vapor diffusion device 8. This device has a sintered disc 9 at the end of line 6 to give a turbulent nitrogen flow, an inner container 10 which is a constant base capillary tube, containing the material to be adsorbed, and a water jacket 11 controlled by a thermostat (not shown) to give a constant temperature which also controls the amount taken up by the nitrogen. Line 12 connects the diffusion device 8 with a selector valve 13. Also connected to the selector valve is a line 14 having a valve 15, which by-passes vapor diffusion device 8 and a line 16 with associated pressure gauge 17 and valve 18 through which pure hydrogen may be fed. This line 16 is only required if the system has to be purged or if hydrogen is required as a pretreatment or carrier gas.

From selector valve 13 a line 19 passes to the sample holder 20, which is a stainless steel tube 2½ inches long and  $\frac{5}{32}$  inch bore, the sample to be tested being held in the tube by quartz wool plugs. A furnace 21 surrounds the holder 20, heated by an electrical winding (not shown). The temperature of the furnace is controlled by a thermostat and thermocouple, the lead of which is shown at 22. From the holder 20 a line 23 passes via a union 38 to a sampling valve 24 and a line 25 from the valve 24 allows gas to flow to atmosphere through a soap film flowmeter 26. A line 27 from the selector valve 13 which by-passes the sample holder 20 can also be connected via union 38 to the sampling valve 24. A line 28 leads from the valve 24 to the hydrogen-flame ionization detector 29. The sampling valve can be operated at regular intervals by a pneumatic cylinder 30 which is in turn activated by a solenoid 31 and a timer 32.

The hydrogen flame-ionization detector is of a known type as described in Gas Chromatography, Third Symposium (Ed. R. P. W. Scott), Butterworth and Co. at page 46. It consists essentially of a source of hydrogen 33 and air 34 giving a hydrogen flame at 35. Gas from the sampling valve 24 is fed via line 28 to the hydrogen flame and changes in the ionization of the surrounding atmosphere are recorded electrically, amplified at 36, and used to actuate a pen recorder 37.

In operation a sample of catalyst is placed in the sample holder 20. Selector valve 13 is manually positioned so that nitrogen line 14 is connected to the holder 20, the nitrogen passing over the catalyst through line 23 to the atmosphere. The furnace 21 is brought up to the desired pretreatment temperature and held for a given period while nitrogen flow is continued. This constitutes the conditioning pretreatment. During this time nitrogen and vapor from line 6 are passing through the selector valve 13 via the by-pass line 27 through the union 38 to the sampling valve 24. Operation of the valve timing device is started so that, at regular intervals, samples of the nitrogen and vapor pass to the detector 29. This enables the composition of the nitrogen feed stream to be determined and adjustment made to the flow valve 7 to give the desired partial pressure of vapor in the nitrogen.

At the end of the conditioning period, and providing the vapor partial pressure is constant, the furnace temperature is adjusted as necessary. When a steady temperature has been reached sampling is stopped and line 27 is disconnected from the union 38 and line 23 connected in its place. The selector valve 13 is then manually operated so as to direct nitrogen and vapor to the holder 20. At the same moment the sampling valve 24 is restarted and samples of the effluent are automatically taken at regular intervals and the detector response, which is a measure of the vapor concentration in the effluent, is recorded. This will be less than the amount fed according to the amount adsorbed on the catalyst and the flow is continued until no more vapor is adsorbed, i.e. the composition of the feed and effluent are the same. Selector valve 13 is then altered again so that pure nitrogen

free of vapor is directed into the holder. Adsorbed vapor is desorbed from the catalyst and recorded in the effluent. When no further vapor is desorbed the test is terminated.

A typical record of a test is shown in FIGURE 2. During the period when nitrogen and vapor are passing, the detector shows initially no response indicating that all the vapor is being adsorbed and none is appearing in the effluent. Vapor gradually appears in the effluent until it reaches a steady state, the amount being recorded at regular intervals. Nitrogen alone is then passed and the amount of vapor desorbed is recorded until the effluent composition is steady. From such a record a quantitative determination of the amount of vapor adsorbed and desorbed can be made. Thus, after a correction for the known dead volume of the apparatus, the amount adsorbed is the difference between the total rectangular area of the adsorption period and the area under the curve formed by the peaks of the regular periodic records. The amount desorbed is the area under the curve formed by the peaks during the desorption section of the record. A quantitative figure for the actual mass of vapor passed during the adsorption period can be obtained from the vapor diffusion device 8, either by direct measurement of the small change of liquid level in the inner container 10 during the adsorption using a travelling microscope, or by calculation according to the formula

$$S = \frac{DMPA}{RTl} \ln \left( \frac{P}{P-p} \right)$$

where

$S$ =mass transfer (g. sec.<sup>-1</sup>)

$D$ =coefficient of gaseous diffusion (cm.<sup>2</sup>/sec.)

$M$ =molecular weight

$R$ =gas constant (erg/deg/mole)

$T$ =absolute temperature

$A$ =cross sectional area of diffusion tube (cm.<sup>2</sup>)

$P$ =pressure at open end of diffusion tube (dyne cm.<sup>-2</sup>)

$p$ =vapor pressure of liquid in diffusion tube (dyne cm.<sup>-2</sup>)

$l$ =length of space above liquid in diffusion tube (cm.)

This gives a correlation between the actual area of the record and the mass of vapor passed and enables the areas to be converted into quantitative figures. The amount desorbed is the reversible adsorption, which can be expressed in  $\mu$ moles/gram of catalyst.

The apparatus and the technique naturally require considerable attention to detail and accuracy in accordance with known analytical procedures beyond the brief details given above. Once the apparatus and techniques have been established, however, the method is rapid and accurate and capable of being used on relatively small samples.

In addition to the discovery that an improved yield-octane number relationship is obtained by the use of a platinum group metal on a low-acidity alumina support, it has been found that the reforming process may be still further improved by the use in combination of such a catalyst and a second catalyst having a platinum group metal disposed on a more acidic support. Catalysts of a platinum group metal on an acidic alumina support are well known in the art, and the acidic alumina may be derived from alumina hydrate precursors which contain predominantly trihydrate aluminas, particularly beta-alumina trihydrate (also known as bayerite).

Where, as is preferred, the acidity of the second catalyst support is conferred by the nature of the alumina itself, a convenient criterion of acidity may be a reversible benzene chemisorption of at least 10  $\mu$ moles/g., and preferably at least 15  $\mu$ moles/g.

Alternatively, acidity may be conferred on the alumina by the addition of halogens, particularly fluorine and chlorine, to the catalyst during its preparation and/or to the reforming reaction zone or zones. Thus, halogen injection may be made to the feed stream just prior to

contact with the more acidic catalyst. The halogen may be present in an amount of from 0.1 to 8% wt. by weight of the total (second) catalyst, particularly 0.1 to 2% wt. However if a halogen-containing catalyst is used, care should be taken to ensure that excessive halogen does not enter the reaction zone or zones containing the low-acidity catalyst, since this may give an undesirable increase in hydrocracking in this zone or zones. Mixtures, having acidic properties, of alumina with at least one other oxide of elements from Groups III and IV of the Periodic Table may also be employed as the catalyst support, for example, mixtures with boria, silica, titania, or zirconia. The oxide or oxides other than alumina are preferably present in amount of from 1 to 25% wt., by weight of the total (second) catalyst.

The platinum group metal content and methods of adding it to the support may be the same as for the low acidity catalyst.

As stated earlier, the feedstock is first contacted with the catalyst having the low acidity support, and then with the second catalyst. It is desirable that no separation of any part of the reaction mixture takes place between contacting the two catalysts. Preferably the pressure and gas flow rate are constant for both catalysts.

The amount of low-acidity catalyst to total catalyst may conveniently be in the range 5 to 90% vol., more particularly 15 to 75% vol. Since in commercial practice reformers have a number of separate reactors in series, for Example 3, the first reactor, and also, if desired, the second reactor can be used for the low-acidity catalyst and the other reactor or reactors for the more acidic catalyst.

The reforming conditions under which the low-acidity catalyst is used may be selected from the following ranges:

Temperature, ° F. ..... 800-1100 (preferably 900-1050).

Pressure, p.s.i.g. ..... 0-1000 (preferably 200-500).

Space velocity, v./v./hr. ..... 0.01-10 (preferably 1-5).

Gas flow rate (recycle or once through), s.c.f./b. ..... Up to 20,000 (preferably 2,000-20,000).

When the process uses both low-acidity and high-acidity catalysts, the process conditions for the acidic catalysts are also selected from the same ranges.

The invention is illustrated by the following examples.

#### EXAMPLE 1

This example, and Example 2 illustrate the preparation of a low acidity alumina-based catalyst and compare results obtained by its use in accordance with one embodiment of the invention with those obtained by the use, separately, of high acidity alumina-based catalysts.

##### Catalyst 1.—*Pseudoboehmite-derived low acidity alumina*

2000 g. of powdered aluminium isopropoxide were slurried into 8 litres of 6 percent weight hydrogen peroxide solution, and stirring continued for 6 days. The slurry was then centrifuged, washed with deionized water to remove most of the hydrogen peroxide, and reslurried in 1 liter of deionized water. 150 ml. of solution containing 7.5 g. of chloroplatinic acid (platinum content about 40 percent weight) were added slowly to the slurry which was vigorously stirred for about 30 minutes. Hydrogen sulphide gas was then bubbled through the slurry for about 1 hour, after which it was centrifuged and washed with about 3 liters of acetone to remove some of the residual water from the filter cake. The partially dried filter cake was then left under vacuum overnight, and finally dried in a forced air oven at 120° C.

The dried hydrate was crushed, pelleted to  $\frac{3}{16}$ " x  $\frac{3}{16}$ ", and granulated to 8-16 mesh. It was then calcined in a muffle furnace for 2 hours at 500° C., cooled in a desicca-

tor and stored in a sealed container until required for use.

*Catalyst 2.—Bayerite-derived high acidity alumina*

2000 g. of aluminium isoproxide were dissolved in 12 liters of Analar benzene, 6 liters of 5 percent weight ammonium hydroxide were added and the mixture stirred vigorously for 1 hour. After this time hydrolysis of the aluminium isoproxide was complete. The benzene layer, containing most of the isopropyl alcohol formed during the reaction, was decanted, and a further 4 liters of 5 percent weight ammonium hydroxide added to the alumina hydrogel slurry. Stirring was continued overnight, after which the slurry was centrifuged, washed with about 8 liters of deionized water, and the filter cake reslurried in 4 liters of deionized water. To homogenize the slurry

10

15

Catalysts 1, 2 and 3 were tested for reforming activity under the following conditions.

|                                    |                                                      |
|------------------------------------|------------------------------------------------------|
| Plant pressure, p.s.i.g.           | 450.                                                 |
| Space velocity, v./v./hr.          | 2.0.                                                 |
| Recycle gas rate, s.c.f./b.        | 20,000.                                              |
| Catalyst mid-bed temperature, ° F. | 930-975.                                             |
| Catalyst charge, ml.               | 250.                                                 |
| Feedstock                          | Dry, desulphurized<br>70°-127° C. gasoline fraction. |

The catalysts were reduced at 900° F. with dry hydrogen for 2 hours before the unit was brought on stream. Test periods were carried out at temperatures of 930° F., 960° F., 975° F. and again at 930° F.

The total on stream time of the test was 110 hours.

The liquid product yields and research octane numbers (clear) of the products are given in Table 2 below.

TABLE 2

| Catalyst | 930° F.            |      | 960° F.            |      | 975° F.            |      | 930° F.            |      |
|----------|--------------------|------|--------------------|------|--------------------|------|--------------------|------|
|          | Yield, percent wt. | RON  | Yield, percent wt. | RON  | Yield, percent wt. | RON  | Yield, percent wt. | RON  |
| 1        | 91.6               | 70.2 | 81.9               | 87.7 | 78.6               | 90.1 | 90.4               | 71.9 |
| 2        | 76.3               | 84.7 | 66.0               | 95.3 | 62.5               | 98.6 | 76.5               | 86.4 |
| 3        | 75.9               | 88.0 | 65.9               | 94.5 | 65.6               | 97.7 | 79.2               | 84.2 |

Yield=Liquid product yield on output basis, corrected to C<sub>5</sub>+ stabilized basis.

RON=Product octane number, research clear, corrected to C<sub>5</sub>+ stabilized basis.

it was passed six times through a colloid mill (using Carborundum stones), the clearance being progressively reduced to 0.001 inch. 1500 ml. of 0.880% ammonia were then added to the thickened slurry with vigorous stirring. The slurry was aged at ambient temperature in a sealed polythene container.

After 10 days ageing, the slurry was centrifuged washed to remove most of the ammonium hydroxide, and the filter cake reslurried in deionized water. 150 ml. of solution containing 8 g. of chloroplatinic acid (platinum content about 40 percent weight) were added slowly, with vigorous stirring, to the alumina hydrogel slurry. After 30 minutes' stirring, hydrogen sulphide gas was bubbled through the slurry for 3/4 hour, and then the platinum-alumina hydrogel was dried in a forced air oven at 120° C.

The platinum-alumina hydrate was pelleted, granulated and calcined in the same way as Catalyst 1.

A further catalyst, Catalyst 3, which was used for comparative test was a commercially available platinum-alumina-halogen catalyst.

Chemical and physical data on the three catalysts are given in Table 1 below.

In addition to yields and octane numbers, the exit gas and stabilizer gas makes were also determined.

A comparison of the results obtained with the three catalysts showed the following differences.

(a) YIELD-OCTANE RELATIONSHIP

The results given in Table 2 are plotted on the accompanying graph FIGURE 3, which plots the C<sub>5</sub>+ liquid product yield against research octane number clear. The graph shows clearly the better yield-octane relationship obtained with Catalyst 1. At 90 RON, for example, the yield advantage is 5% wt. and at 78% wt. yield the octane number advantage is 5 numbers.

(b) EXIT STABILIZER GAS MAKES

At any given octane number, the exit gas make and the hydrogen content of that gas were highest for Catalyst 1 and lowest for Catalyst 2. At 90 RON for example the hydrogen make was

|            | S.c.f./b. |
|------------|-----------|
| Catalyst 1 | 700       |
| Catalyst 2 | 330       |
| Catalyst 3 | 490       |

TABLE 1

| Catalyst                                                 | 1                                      | 2                                                              | 3           |
|----------------------------------------------------------|----------------------------------------|----------------------------------------------------------------|-------------|
| Composition:                                             |                                        |                                                                |             |
| Platinum, percent wt.                                    | 0.55                                   | 0.66                                                           | 0.739       |
| Chlorine, percent wt.                                    | 0.62                                   | 0.51                                                           | 0.29        |
| Sodium, percent wt.                                      | 0.002                                  | 0.006                                                          |             |
| Potassium, percent wt.                                   | 0.005                                  | 0.006                                                          |             |
| Fluorine, percent wt.                                    | Nil                                    | Nil                                                            |             |
| Surface Area m <sup>2</sup> /g.                          | 261                                    | 365                                                            |             |
| Pore Volume, ml./g.                                      | 0.24                                   | 0.31                                                           | 0.63        |
| X-ray Data:                                              |                                        |                                                                |             |
| Pt-Alumina hydrate                                       | Pseudobohemite                         | Mainly bayerite with a little norstrandite and pseudobohemite. |             |
| Pt-Alumina (after calcination for 2 hr. at 1,020° F.).   | Eta-alumina of small crystalline size. | Eta-alumina                                                    | Eta-alumina |
| Benzene Chemisorption Data:                              |                                        |                                                                |             |
| Benzene/Pt atom ratio <sup>1</sup>                       | 0.141                                  | 0.104                                                          | 0.23        |
| Benzene adsorption on alumina base, <sup>2</sup> μmol/g. | 3.5                                    | 16                                                             | 10          |

<sup>1</sup> Irreversible benzene chemisorption at 150° C., on pre-reduced Pt-alumina catalyst.

<sup>2</sup> Reversible benzene chemisorption at 193° C. on the alumina base.

The stabilizer gas make showed the reverse trend, the figures at 90 RON being

|            | S.c.f./b. |
|------------|-----------|
| Catalyst 1 | 300       |
| Catalyst 2 | 470       |
| Catalyst 3 | 380       |

These results can be interpreted as showing that Catalyst 1 has a low activity for hydrocracking (a hydrogen-consuming and gaseous hydrocarbon-producing reaction) and a good activity for dehydrocyclization and dehydrogenation (hydrogen-producing reactions).

#### EXAMPLE 2

The pseudo-boehmite based platinum-alumina (Catalyst 1) was tested for reforming activity under more severe operating conditions to produce C<sub>5</sub>+ reformate of 95 and 100 RON (clear).

The following operating conditions were employed:

| Liquid product RON (Clear) -----        | 94-95                                                     | 99-100 |
|-----------------------------------------|-----------------------------------------------------------|--------|
| Catalyst mid-bed temperature, ° F ----- | 975                                                       | 995    |
| Space velocity, v./v./hr -----          | 2.0                                                       | 1.4    |
| Plant pressure, p.s.i.g -----           | 450                                                       |        |
| Gas recycle rate, s.c.f./b -----        | 20,000                                                    |        |
| Feedstock -----                         | Dry, desulphurized, 80-160° C.<br>ASTM gasoline fraction. |        |

The catalyst was reduced at 900° F. with dry hydrogen for 2 hours before the unit was brought on stream.

The following results were obtained:

##### (a) OPERATION AT 95 OCTANE NUMBER LEVEL

| Hours on stream -----                 | 214-220 | 405-411 |
|---------------------------------------|---------|---------|
| RON (Clear) -----                     | 94.6    | 94.7    |
| Liquid yield, percent wt -----        | 77.4    | 77.6    |
| Exit gas, s.c.f./b -----              | 910     | 899     |
| H <sub>2</sub> content, percent ----- | 75      | 73.5    |
| Stabilizer gas, s.c.f./b -----        | 262     | 270     |

##### (b) OPERATION AT 100 OCTANE NUMBER LEVEL

| Hours on stream -----                 | 669-675 | 837-843 | 1,000-1,010 |
|---------------------------------------|---------|---------|-------------|
| RON (Clear) -----                     | 99.7    | 99.8    | 99.3        |
| Liquid yield, percent wt -----        | 64.1    | 64.2    | 63.4        |
| Exit gas, s.c.f./b -----              | 972     | 919     | 934         |
| H <sub>2</sub> content, percent ----- | 64.0    | 64.2    | 63.8        |
| Stabilizer gas, s.c.f./b -----        | 428     | 428     | 417         |

TABLE 3

| Catalyst -----                                           | Case A |       |      |      | Case B |       |      |      | Case C |      |      |      | Case D |      |      |      |
|----------------------------------------------------------|--------|-------|------|------|--------|-------|------|------|--------|------|------|------|--------|------|------|------|
|                                                          | 1      | 2     | 3    | 4    | 1      | 2     | 3    | 4    | 1      | 2    | 3    | 4    | 1      | 2    | 3    | 4    |
| Test Period Number -----                                 | 930    | 959   | 901  | 943  | 930    | 959   | 900  | 929  | 931    | 960  | 900  | 930  | 959    | 984  | 1010 | 960  |
| Catalyst mid-bed temperature, ° F -----                  | 73.7   | 69.4  | 82.9 | 72.0 | 75.4   | 69.4  | 84.5 | 75.3 | 80.5   | 75.5 | 88.4 | 80.7 | 84.0   | 78.1 | 73.5 | 84.2 |
| Stabilized Reformate Product:                            |        |       |      |      |        |       |      |      |        |      |      |      |        |      |      |      |
| Research Octane Number, Clear -----                      | 95.8   | 101.4 | 86.4 | 97.8 | 96.6   | 102.3 | 86.4 | 95.9 | 92.0   | 99.1 | 80.5 | 91.3 | 92.1   | 95.6 | 98.9 | 90.0 |
| Reformate yield, percent wt -----                        |        |       |      |      |        |       |      |      |        |      |      |      |        |      |      |      |
| Available H <sub>2</sub> production, s.c.f./b -----      | 672    | 743   | 572  | 660  | 603    | 772   | 615  | 689  | 732    | 758  | 610  | 730  | 689    | 761  | 738  | 694  |
| H <sub>2</sub> content of recycle gas, percent mol ----- | 66.2   | 62.9  | 77.6 | 66.3 | 72.9   | 65.9  | 79.2 | 72.5 | 78.5   | 72.5 | 83.5 | 80.5 | 76.0   | 73.0 | 67.1 | 78.3 |

The run was voluntarily terminated at 1,011 HOS (7.8 bbl./lb.)

Despite the very severe operating conditions, the run was characterized by the very high stability of operation. No noticeable activity decline was observed while processing at either 95 or 100 octane number level.

#### EXAMPLE 3

This example gives results obtained by the use in combination of a low acidity alumina based catalyst together with a high acidity alumina based catalyst, according to the second embodiment of the invention.

The two catalysts were Catalyst 1, prepared as described in Example 1, and with the physical and chemical data given in Table 1, and a commercial reforming catalyst consisting of 0.58% wt. platinum and 0.8% wt. chlorine on an acidic alumina having a reversible benzene chemisorption of 17 μmols/g.

Four combinations were examined, viz.:

|                 |                                         |
|-----------------|-----------------------------------------|
| 25 Case A ----- | Commercial catalyst only.               |
| Case B -----    | 20% catalyst 1+80% commercial catalyst. |
| Case C -----    | 60% catalyst 1+40% commercial catalyst. |
| 30 Case D ----- | Catalyst 1 only.                        |

For Case B, as an example, the two catalysts were placed in the reactor, the first (Catalyst 1) at the top of the bed and the second below it, and a downflow feed system was used. An activity test was carried out at a series of temperatures and under the following operating conditions:

|                                          |                                                   |
|------------------------------------------|---------------------------------------------------|
| 40 Temperature -----                     | 930, 960, 900° F.                                 |
| Pressure -----                           | 450 p.s.i.g.                                      |
| Space velocity (on total catalyst) ----- | 2.0 v./v./hr.                                     |
| Gas flow rate -----                      | 20,000 s.c.f./b.                                  |
| 45 Feedstock -----                       | Dry desulphurized 90-140° C. ASTM light gasoline. |

The same operating procedure was applied using the catalyst combination of Case A and of Case C, the results being summarized in Table 3. Table 3 also shows the results obtained with Case D. In this instance the conditions are similar to those for Cases A to C, except that the mid-bed temperatures are higher in order to bring the product octane numbers up to the required level.

Referring now to the accompanying drawings, the research octane number, clear, is plotted against the C<sub>5</sub>+ liquid product yield for Cases A to D in FIG. 4, the research octane number, clear against the stabilizer gas make in FIG. 5a and the available hydrogen production in FIG. 5b.

Table 4 below compares Cases B, C, and D with Case A, and gives, in addition to the yield advantage at given octane numbers, the temperature penalty at these octane numbers.

It will be seen from FIG. 4 and Table 4 that Case B gives approximately a 1.5% yield advantage over Case A at all octane numbers with no temperature penalty. If a temperature penalty of 15-20° F. is acceptable, then Case C provides a yield advantage over Case A that increases with increasing octane number. Case D has a yield advantage over Case A at all octane numbers at least up to 100, but the temperature penalty is higher.

FIGURE 5a shows that each of Cases B to D produced more hydrogen at a given octane number than Case A, and in conjunction with the stabilizer gas production, indicated in FIGURE 5b this can be considered to show that each of the combined catalysts has a higher dehydrocyclization/dehydrogenation activity and a lower hydrocracking activity than the known high acidity catalyst when used alone.

TABLE 4.—COMPARISON OF CASES B, C AND D WITH CASE A

| RON Clear                                           | 90  | 95  | 100 |
|-----------------------------------------------------|-----|-----|-----|
| Reformate Yield Advantage over Case A, percent wt.: |     |     |     |
| B                                                   | 2   | 1.5 | 1.5 |
| C                                                   | 2.5 | 3.5 | 4.5 |
| D                                                   | 6   | 4   | 2   |
| Temperature Penalty, ° F.:                          |     |     |     |
| B                                                   | Nil | Nil | Nil |
| C                                                   | 15  | 20  | 20  |
| D                                                   | 45  | 50  | 65  |

I claim:

1. A process for the catalytic reforming of hydrocarbons which comprises contacting a C<sub>5</sub>-204° C. hydrocarbon fraction, in the presence of a hydrogen-rich gas, with a catalyst comprising platinum on a support consisting of an alumina having a reversible benzene chemisorption of up to 5 μmols/g., at a temperature of from 800-1100° F., a pressure of from 0-1000 p.s.i.g., a space velocity of from 0.01-10 v./v./hr., and a gas flow rate of up to 20,000 s.c.f./b.

2. A process as claimed in claim 1, wherein the catalyst support consists of an alumina having a reversible benzene chemisorption of from 0.3-5 μmols/g.

3. A process as claimed in claim 1, wherein the temperature is 900-1050° F., the pressure is 200-500 p.s.i.g., the space velocity is 1-5 v./v./hr., and the gas flow rate is 2000-20,000 s.c.f./b.

4. A process as claimed in claim 1, wherein the said alumina is derived from a pseudoboehmite alumina hydrate precursor obtained by hydrolysis of an aluminium alcoholate at a temperature of less than 70° C.

5. A process as claimed in claim 1, wherein the platinum content of the catalyst is 0.01-5% weight.

6. A process for the catalytic reforming of hydrocarbons, which comprises contacting a C<sub>5</sub>-204° C. hydrocarbon fraction, in the presence of a hydrogen-rich gas with a first catalyst comprising platinum on a support consisting of an alumina having a reversible benzene chemisorption of up to 5 μmols/g., and then with a second catalyst comprising platinum on a support consisting of an alumina having a reversible benzene chemisorption of at least 10 μmols/g., at a temperature of from 800-1100° F., a pressure of from 0-1000 p.s.i.g., a space veloc-

ity of from 0.01-10 v./v./hr., and a gas flow rate of up to 20,000 s.c.f./b.

7. A process as claimed in claim 6, wherein the support of the said first catalyst consists of an alumina having a reversible benzene chemisorption of from 0.3-5 μmols/g.

8. A process as claimed in claim 6, wherein said first catalyst constitutes from 15-75% vol. of the total volume of the first and second catalysts.

9. A process as claimed in claim 6, wherein the temperature is 900-1050° F., the pressure is 200-500 p.s.i.g., the space velocity is 1-5 v./v./hr., and the gas flow rate is 2000-20,000 s.c.f./b.

10. A process as claimed in claim 6, wherein the alumina support of the said first catalyst is derived from a pseudoboehmite alumina hydrate precursor obtained by hydrolysis of an aluminium alcoholate, at a temperature of less than 70° C., and wherein the alumina support of the said second catalyst is derived from a precursor consisting predominantly of beta-alumina trihydrate also known as bayerite.

11. A process as claimed in claim 6, wherein the total platinum content of the first and second catalysts is 0.01-5% weight.

12. A process for the catalytic reforming of hydrocarbons, which comprises contacting a C<sub>5</sub>-204° C. hydrocarbon fraction, in the presence of a hydrogen-rich gas, with a first catalyst comprising platinum on a support consisting of an alumina having a reversible benzene chemisorption of up to 5 μmols/g., and then with a second catalyst comprising platinum on a support consisting of a mixture of alumina with at least one other oxide of elements selected from Groups III and IV of the Periodic Table, said second catalyst being more acidic than said first catalyst, at a temperature of from 800-1100° F., a pressure of from 0-1000 p.s.i.g., a space velocity of from 0.01-10 v./v./hr., and a gas flow rate of up to 20,000 s.c.f./b.

13. A process as claimed in claim 12, wherein the support of the said first catalyst consists of an alumina having a reversible benzene chemisorption of from 0.3-5 μmols/g.

14. A process as claimed in claim 12, wherein the support of the said second catalyst comprises from 1-25% weight, by weight of said other oxides.

15. A process as claimed in claim 12, wherein said first catalyst constitutes from 15-70% vol. of the total volume of the first and second catalysts.

16. A process for the catalytic reforming of hydrocarbons, which comprises contacting a C<sub>5</sub>-204° C. hydrocarbon fraction, in the presence of a hydrogen-rich gas, with a first catalyst comprising platinum on a support consisting of an alumina having a reversible benzene chemisorption of up to 5 μmols/g., and then with a second catalyst comprising platinum on a support consisting of alumina and from 0.1-8% weight of halogen by weight of the said second catalyst, said second catalyst being more acidic than said first catalyst, at a temperature of from 800-1100° F., a pressure of from 0-1000 p.s.i.g., a space velocity of from 0.01-10 v./v./hr., and a gas flow rate of up to 20,000 s.c.f./b.

17. A process as claimed in claim 15, wherein the support of the said first catalyst consists of an alumina having a reversible benzene chemisorption of from 0.3-5 μmols/g.

18. A process as claimed in claim 15, wherein said first catalyst constitutes from 15-75% vol. of the total volume of the first and second catalysts.

19. A process for the catalytic reforming of hydrocarbons, which comprises contacting a C<sub>5</sub>-204° C. hydrocarbon fraction, in the presence of a hydrogen-rich gas, with a first catalyst comprising platinum on a support consisting of an alumina having a reversible benzene chemisorption of from 0.3-5 μmols/g., and then with a second catalyst comprising platinum on a support consisting of an alumina having a reversible benzene chemisorption of at least 10 μmols/g., at a temperature of from 900-

1050° F., a pressure of from 200-500 p.s.i.g., a space velocity of from 1-5 v./v./hr., and a gas flow rate of from 2000-20,000 s.c.f./b., said first catalyst constituting from 15-75% vol. of the total volume of the first and second catalysts, the total platinum content of the first and second catalysts being 0.01-5% weight, the alumina support of the first catalyst being derived from a pseudoboehmite alumina hydrate precursor obtained by hydrolysis of an aluminium alcoholate at a temperature of less than 70° C., and the alumina support of the second catalyst being derived from a precursor consisting predominantly of beta-<sup>5</sup> alumina trihydrate also known as bayerite.

## References Cited

## UNITED STATES PATENTS

|           |         |                          |         |
|-----------|---------|--------------------------|---------|
| 2,796,326 | 6/1957  | Kimberlin et al. _____   | 208—138 |
| 2,885,345 | 5/1959  | Hemminger et al. _____   | 208—65  |
| 2,903,418 | 9/1959  | Kirshenbaum et al. _____ | 208—38  |
| 2,908,628 | 10/1959 | Schneider et al. _____   | 208—65  |
| 3,038,784 | 6/1962  | Torkar et al. _____      | 23—143  |

DELBERT E. GANTZ, Primary Examiner.

H. LEVINE, Assistant Examiner.

UNITED STATES PATENT OFFICE  
CERTIFICATE OF CORRECTION

Patent No. 3,328,286

June 27, 1967

Paul Anthony Lawrance

It is hereby certified that error appears in the above numbered patent requiring correction and that the said Letters Patent should read as corrected below.

In the heading to the printed specification, line 6, for "The British Petroleum Company" read -- The British Petroleum Company Limited --; column 7, line 47, after "centrifuged" insert a comma; columns 9 and 10, TABLE 3, seventeenth column, line 1, for "90.0" read -- 90.6 --; column 12, line 46, for "15-70%" read -- 15-75% --.

Signed and sealed this 29th day of October 1968.

(SEAL)

Attest:

Edward M. Fletcher, Jr.

Attesting Officer

EDWARD J. BRENNER  
Commissioner of Patents